

Nov. 22, 1938.

R. H. IMES ET AL

2,137,617

ELECTRICAL CONTACT AND METHOD OF MAKING THE SAME

Filed March 4, 1936



INVENTORS  
Robert H. Imes  
BY Hal F. Truth  
Barrett C. Smith  
ATTORNEY

## UNITED STATES PATENT OFFICE

2,137,617

ELECTRICAL CONTACT AND METHOD OF  
MAKING THE SAMERobert H. Imes and Hal F. Fruth, Indianapolis,  
Ind., assignors to P. R. Mallory & Co., Inc., In-  
dianapolis, Ind., a corporation of Delaware

Application March 4, 1936, Serial No. 67,010

13 Claims. (Cl. 29—155.55)

This invention relates to electrical contacts and methods of making the same.

An object of the invention is to improve the methods of making electrical contacts.

5 Another object is to produce an improved electrical contact.

Other objects of the invention will be apparent from the following description and accompanying drawing taken in connection with the 10 appended claims.

The invention comprises the features of construction, combination of elements, arrangement of parts, and methods of manufacture and operation referred to above or which will be 15 brought out and exemplified in the disclosure hereinafter set forth, including the illustrations in the drawing, the scope of the invention being indicated in the appended claims.

For a fuller understanding of the nature and 20 objects of the invention as well as for specific fulfillment thereof, reference should be had to the following detailed description taken in connection with the accompanying drawing in which:

25 Figure 1 is a face view of an electrical contact made according to the present invention;

Figure 2 is a section on the line 2—2 of Figure 1;

Figure 3 is a face view of a steel blank used in 30 fabricating contacts of the kind shown in Figure 1;

Figure 4 is a section on the line 4—4 of Figure 3;

Figure 5 is a section through a preliminary 35 assembly comprising the steel blank and a disc of contact metal;

Figure 6 is a section through the assembly after fusion of the contact metal to the steel 40 backing;

Figure 7 shows the coining operation; and

Figure 8 shows the operation of punching the contact from the steel strip on which it was 45 formed.

While a preferred embodiment of the invention 50 is described herein, it is contemplated that considerable variation may be made in the method of procedure and the construction of parts without departing from the spirit of the invention. In the following description and in the claims, parts will be identified by specific names for convenience, but they are intended to be as generic in their application to similar parts as the art will permit.

An important use of the present invention is 55 in the production of steel-backed silver-faced

contacts wherein a contact face of silver or a silver alloy is integrally united to a steel backing. In prior practice such contacts have been made by punching the contact discs out of bimetallic sheet stock consisting of a sheet of steel having a uniform layer of silver welded to its surface. It will be readily apparent that this procedure is wasteful and uneconomical because of the fact that a sizeable proportion of the silver is left on the scrap material from which the contact discs have been punched. These prior methods, therefore, require a considerable investment in material which is converted into scrap which requires further processing in order to recover the precious metal. The present invention provides an improved method of making contacts which does not have these objections.

Referring to the drawing, a silver-faced contact 10 is illustrated in Figures 1 and 2 and the method of making the contact is illustrated in Figures 3 to 8. In this method a strip of sheet steel 11 is run through a stamping machine or punch press wherein a series of annular grooves 12 are stamped in the strip. In the same operation an indentation 13 is formed on the same face with the annular groove and preferably concentric therewith. A corresponding projection 14 is thereby provided on the opposite face of the strip. A series of locating or centering holes 15 is also punched in the strip in a line parallel to the line of centers of the annular grooves, the centering holes being spaced apart by the same distances as the annular grooves. After the above operation the steel strip will have the form shown in Figures 3 and 4.

The next step in the procedure is to place a piece 16 of the contact metal, such as silver, on or in contact with the steel strip within the area enclosed by each annular groove 12. The pieces each contain a definite predetermined quantity of metal and may be in the form of discs punched from sheet, slugs punched from wire or small pieces formed in other ways.

The steel strip 11, carrying pieces 16 in contact, is then passed through a furnace where the assembly is heated to a temperature above the melting point of the silver or silver alloy. When the silver is in the molten condition it flows out over the surface of steel strip 11 until it reaches the inner edge of groove 12, where the flow is stopped, probably because the surface tension of the molten silver is greater than the attraction of the silver for the steel at this point. Should the silver flow over the inner edge of the groove it will be stopped at the outer edge.

There results a body of molten silver which solidifies, on removal from the furnace, into a solid layer 17 adhering to the steel backing within the area bounded by the annular groove, 5 the silver layer having a convex circular face 18 (Fig. 6).

The convex face 17 may, in some instances, be suitable for use as a contact face without extra treatment. It is generally desirable, however, to 10 insure perfect uniformity of dimensions and to obtain the exact radius of curvature desired, to coin the surface. This is accomplished, as indicated in Figure 7, by a pair of punches 19 and 20 held in a suitable pressing arrangement. 15 Punch 19 has a face shaped to receive the projection 14 on the back of the strip and punch 20 has a face 30 of the curvature necessary to apply the desired radius 21 to the silver face. In the coining operation the contact can be centered with respect to the punches by one or more 20 locating pins 22 adapted to fit into holes 15.

The finished contacts are punched from strip 11 by a punch 23, having a face shaped to receive projection 14, in cooperation with a die 24. 25 The punch 23 and die 24 have a diameter 26 slightly less than that of annular ring 12 so that some of the silver contact metal is drawn down around the sides of the punched disc to cover the edges as is apparent from Figure 2. In 30 the punching operation locating pin 25 co-operates with hole 15 in the steel strip to center the contact in the die.

The finished contact 10 is thereby produced having a circular silver face with a curvature 35 21, the silver face being integrally attached to a steel backing disc 27 and extending down over the edges thereof. The steel disc 27 also has welding projection 14 whereby the contact can be electrically welded to a switch spring, circuit breaker armature, breaker arm, relay armature or any other metal part on which it is desired to provide contacts.

It will be obvious that other contact materials, 40 in some instances, can be used in place of silver and other backing materials can be used in place of steel. Composite facings may also be formed. The metal in contact with the backing must, of course, be of lower melting point than the backing metal.

50 While the present invention, as to its objects and advantages, has been described herein as carried out in specific embodiments thereof, it is not desired to be limited thereby but it is intended to cover the invention broadly within the 55 spirit and scope of the appended claims.

What is claimed is:

1. The method of making an electric contact which comprises providing an annular groove in one face of a sheet of backing metal, placing a 60 quantity of lower melting point contact metal in contact with said face in the area surrounded by said groove, heating the assembly thus produced to a temperature above the melting point of said contact metal, whereby it is fused to said 65 backing metal, cooling said assembly and punching a disc from an area of said backing metal sheet including at least part of the area within said annular groove, said groove serving to limit the flow of the melted contact metal during said heating.

70 2. The method of making an electric contact which comprises providing a groove in one face of a backing metal member, said groove enclosing a portion of the area of said surface, placing 75 ing contact metal of lower melting point than

said backing metal against said portion, heating said assembly above the melting point of said contact metal but below the melting point of said backing metal, and cooling the integral assembly thus produced, said groove serving to limit the flow of the melted contact metal during 5 said heating.

3. The method of making an electric contact which comprises providing a groove in one face of a metal backing member, said groove enclosing a portion of the area of said face so as to prevent the flow of molten metal of lower melting point than the backing metal away from said area, placing facing metal in contact with said area, at least a portion of said facing metal being suitable for a contact facing and at least a portion of said facing metal being of lower melting point than said backing metal, heating the assembly thus produced above the melting point of said lower melting point metal but below the 20 melting point of said backing metal whereby said lower melting metal will fuse to the surface of said backing metal within said area, and cooling the integral assembly thus produced.

4. The method of making an electrical contact 25 assembly which comprises forming a moat in a face of a backing metal member, placing a lower melting metal in contact with said face inside said moat, heating to fuse said lower melting metal and cooling to solidify the integral 30 assembly thus produced, said moat serving to limit the flow of the melted contact metal during said heating.

5. The method of making an electrical contact 35 which comprises stamping a circular groove in a face of a backing metal member, placing a piece of contact metal of lower melting point than said backing metal within the area enclosed by said groove, heating the assembly to a temperature high enough to melt said lower 40 melting metal only, and cooling the integral assembly thus produced, said groove serving to limit the flow of the melted contact metal during said heating.

6. The method of making an electrical contact 45 which comprises stamping a moat in a face of a backing metal member, placing a piece of silver metal within the area enclosed by said moat, heating the assembly sufficiently to fuse said silver metal without fusing said backing metal, 50 then cooling the assembly below the melting point of said silver metal, said moat serving to limit the flow of the fused silver metal during said heating.

7. The method of making an electrical contact 55 which comprises stamping a circular groove on one face of a piece of sheet steel, placing a piece of silver metal within the area enclosed by said groove, and heating the assembly to fuse the silver to the steel, said groove serving 60 to limit the flow of the fused silver metal during said heating.

8. The method of making an electrical contact which comprises stamping a circular groove on one face of a piece of sheet steel and raising a 65 welding projection on the other face opposite the area enclosed by said circular groove, placing a quantity of silver in contact with the area enclosed by the circular groove, heating the assembly sufficiently to fuse said silver to said area 70 and cooling the integral assembly thus produced, said groove serving to limit the flow of the fused silver during said heating.

9. The method of making an electrical contact which comprises stamping a circular groove on 75

one face of a piece of sheet backing metal, fusing a body of silver metal to said face within the area enclosed by said groove, and punching a bi-metal disc from the silver-backing metal assembly, said groove serving to limit the flow of the fused silver metal during said heating.

10. The method of making an electrical contact which comprises stamping a circular groove on one face of a piece of sheet backing metal, fusing a body of silver metal to said face within the area enclosed by said groove, coining a contact face on said silver metal and punching a bi-metal contact from the assembly, said groove serving to limit the flow of said silver metal during fusing.

11. The method of making an electrical contact which comprises stamping a circular groove on one face of a piece of sheet steel, raising a welding projection on the other face of said sheet opposite the area enclosed by said groove, fusing a body of silver metal to said face within the area enclosed by said groove, coining a contact face on said silver metal and punching a bi-metal contact disc from an area including said silver and said welding projection, said groove serving to limit the flow of said silver metal during fusing.

12. A blank for producing a contact backing comprising a strip of sheet metal having a row of locating holes punched therein, said row being on a line parallel to one edge of said strip, said strip also having a row of annularly grooved portions parallel to said holes.

13. The method of making a bimetal electric contact disk having a curved edge, without waste of the contact metal facing, which comprises integrally securing a layer of contact metal to a sheet metal backing in an area corresponding to an individual contact surrounded by an area of backing metal substantially free from contact metal and then punching said bimetal contact disc out of said sheet metal backing by severing said backing along a line substantially at the boundary of the area to which said contact metal is secured and simultaneously drawing said contact metal down over the edge of the backing along the curved edge of said disc thereby to produce said bimetal contact having a curved edge and with the entire face and edge thereof covered with contact metal.

ROBERT H. IMES. 25  
HAL F. FRUTH.